

## UNITED STATES PATENT OFFICE.

HEINRICH SPECKETER AND OSKAR H. WEBER, OF GRIESHEIM-ON-THE-MAIN, GERMANY, ASSIGNORS TO THE FIRM OF CHEMISCHE FABRIK GRIESHEIM ELECTRON, OF FRANKFORT-ON-THE-MAIN, GERMANY.

## MANUFACTURE OF ALKALI METALS.

SPECIFICATION forming part of Letters Patent No. 730,979, dated June 16, 1903.

Application filed April 17, 1902. Serial No. 103,450. (No specimens.)

To all whom it may concern:

Be it known that we, HEINRICH SPECKETER and OSKAR H. WEBER, subjects of the German Emperor, residing and having our post-office address at 1 Bahnstrasse, Griesheim-on-the-Main, Germany, have invented certain new and useful Improvements in the Manufacture of Alkali Metals, of which the following is a specification.

This invention relates to a process of manufacture of metals of the alkalies by causing metallic aluminium to act upon the fluorine compounds of the corresponding alkali metal.

The mode of action of aluminium of the alkali fluorides has not hitherto been made known. It was already known through the discovery of Wöhler that by the action of metallic sodium on the chlorid of aluminium metallic aluminium was obtained. This is the old process of manufacture of aluminium. With fluorides it is quite the reverse, the reaction taking place in accordance with the following equation:



In consequence besides potassium a double fluorid of aluminium and potassium is obtained. The aluminium does not act on this double salt and does not cause potassium to become free therefrom. The reaction takes place at the melting-point of the potassium fluorid, the potassium distilling off and being obtained pure. The process when using aluminium is entirely free from danger, and it is the only one in which no explosive compound of potassium and carbon oxid is produced. Moreover, the residue of the double

fluorid of aluminium and potassium can be worked again into potassium fluorid. If silico potassium fluorid be used at the beginning, silicium is one of the by-products.

The process is best carried out as follows: In a retort or other suitable vessel ten kilograms of aluminium are heated with the corresponding quantity of potassium fluorid. The aluminium is preferably in the size of large pieces, because if it were in the form of powder the reaction would be too violent and an entrainment of the molten residue would occur. At the melting-point of potassium fluorid the reaction takes place and goes on smoothly until the potassium is entirely displaced. The potassium is collected in a suitable receiver. The residue of the double fluorid of aluminium and fluorid is treated with caustic potash. The resulting potassium fluorid can be used again in a further operation, while the aluminium hydroxid is used again in the aluminium process.

We claim—

The herein-described process of producing alkali metal by heating a mixture of aluminium and alkali fluorid in a suitable distilling apparatus, substantially as and for the purpose set forth.

In testimony whereof we have signed our names to this specification in the presence of two subscribing witnesses.

HEINRICH SPECKETER.  
OSKAR H. WEBER.

Witnesses:

FRANZ HASSLACHER,  
MICHAEL VOLK.